

1

3,385,676

BERYLLIUM PRODUCT COMPRISED OF BERYLLIUM PARTICLES COATED WITH A METAL BERYLLIDE

Charles J. Havel, Allentown, Pa., assignor to The Beryllium Corporation, Reading, Pa., a corporation of Delaware

No Drawing. Original application June 18, 1965, Ser. No. 465,167, now Patent No. 3,298,829, dated Jan. 17, 1967. Divided and this application Sept. 13, 1966, Ser. No. 594,303

3 Claims. (Cl. 29—182.2)

**ABSTRACT OF THE DISCLOSURE**

Beryllium metal shapes formed from beryllium metal particles having metal coating thereon which form beryllides, when subjected to heat and pressure, around each particle and at the interface of each beryllium particle.

The beryllium particles are of a size from 4 to 74 microns, and the coating can be any metal such as chromium, copper, nickel, columbium, molybdenum, cobalt or iron.

This application is a divisional application of Ser. No. 465,167, filed June 18, 1965 now Patent No. 3,298,829.

This invention relates to high strength beryllium and processes of preparing the same.

More specifically, it deals with a process of preparing a beryllium metal having superior elastic modulus, high precision elastic limit, and high tensile strength.

It is an object of the present invention to set forth a new process for producing a beryllium metal having high strength.

Another object of the present invention is to produce a beryllium metal having superior elastic modulus, high precision elastic limit, and high tensile strength which will not experience grain growth during fabrication.

A further object of the instant invention is to set forth a process of producing high strength beryllium alloys wherein the alloy is characterized by a beryllide of the alloying metal at the interface between the particles, and surrounding each particle of beryllium powder so as to inhibit grain growth and reinforce the beryllium matrix.

A more specific object of the instant invention is to set forth a process whereby beryllium powder is coated with a thin coating of a metal which will form a beryllide when pressed into shape under heat.

Other objects and advantages of the invention will become more apparent from the following detailed description and examples.

It has been found that high strength beryllium metal can be formed without sacrificing low bulk density and at the same time having superior elastic modulus, high precision elastic limit, and high tensile strength by coating beryllium powder with a metal capable of forming a beryllide and subsequently hot-pressing the powders to form the new beryllium metal.

The beryllium powder used is of a size of about 4 to 74 microns, but preferably in the order of 4 to 15 microns. This powder is coated with a metal capable of forming a beryllide in any suitable manner, such as for example in the process disclosed in copending application Ser. No. 442,240, now filed Mar. 22, 1965, which is a continuation-in-part of application Ser. No. 260,857, now abandoned. In practice, coatings of up to 50 angstroms have been found suitable. This powder when subjected to pressure and heat forms a beryllide on the surface of each individual particle and at the interface between particles which inhibits grain growth and reinforces the beryllium matrix.

2

Typical of the metals which form beryllides are chromium, copper, nickel, columbium, molybdenum, cobalt and iron. The pressure can vary from 350 pounds per square inch to 2000 pounds per square inch, and the temperature for pressing may vary between 1900° F. to 2200° F. The pressure and temperature utilized as well as the duration of pressing may vary dependent upon the physical characteristics, such as size of the shape being produced.

Some typical examples illustrating the compositions, processes and characteristics of the beryllium metal are the following.

**EXAMPLE I**

15 Nominal 11 micron beryllium powder was vacuum hot-pressed at 2000° F. and 2000 p.s.i.

The chemistry of both the treated powder and the resultant pressing are:

| Constituent | By Analysis, percent |             |
|-------------|----------------------|-------------|
|             | Treated Powder       | Hot Pressed |
| BeO         | 0.5<br>(X-ray diff.) | 4.59        |
| C           | 0.274                | 0.231       |
| Fe          | 0.130                | 0.110       |
| Al          | 0.029                | 0.040       |
| Mg          | 0.111                | 0.095       |
| Ni          | 0.016                | 0.017       |
| Cr          | 0.190                | 0.210       |
| Si          | 0.031                | 0.055       |
| P           | 0.400                | 0.035       |
| Be          | (1)                  | (1)         |
| 1 Balance.  |                      |             |

Example I when hot-pressed and tested gave the following properties:

| Test Direction | U.T.S.<br>K.s.i. | .2% Y.S. | Percent<br>El. | 1u. in.<br>PEL | 2u. in.<br>PEL |
|----------------|------------------|----------|----------------|----------------|----------------|
| 1T             | 179.6            | Nil      | Nil            | 22,125<br>(2)  |                |
| 1L             | 163.4            | Nil      | Nil            | 29,750         | 37,700         |
| 2T             | 3100.0           | Nil      | Nil            | 15,000         | 43,000         |
| 2L             |                  | Nil      | Nil            | 19,000<br>(2)  |                |
| 3T             | 3104.0           | Nil      | Nil            |                |                |
| 3L             | 3103.0           | Nil      | Nil            |                |                |

<sup>1</sup> Tested with extensometer, premature notch failure. Modulus equals  $5.6 \times 10^{-6}$  and  $52.8 \times 10^{-6}$  respectively.

<sup>2</sup> Not determined due to gage slippage.

<sup>3</sup> Tested without extensometer.

L=Longitudinal specimen.

T=Transverse specimen.

Some other examples showing beryllium metals in which the powders were coated with chromium are the following:

TABLE I.—TYPICAL CHEMISTRY OF Be-Cr

| Constituent | Example No.<br>II | Example No.<br>III |
|-------------|-------------------|--------------------|
| BeO         | 4.19              | 5.68               |
| C           | .268              | .438               |
| Fe          | .113              | .127               |
| Al          | .027              | .034               |
| Mg          | .095              | L .001             |
| Ni          | .015              | L .001             |
| Cr          | .210              | .235               |
| Si          | .027              | .039               |
| P           | (1)               | (1)                |
| Be          |                   |                    |

NOTE.—L indicates less than.

60 <sup>1</sup> Balance.

TABLE II.—MECHANICAL PROPERTIES OF Be-Cr (AS PRERESSED)

|         | U.T.S.,<br>K.s.i. | 1 micro in.<br>PEL, p.s.i. | 2 micro inches<br>PEL, p.s.i. |
|---------|-------------------|----------------------------|-------------------------------|
| No. I   | 104.0             | 26,500                     | 29,750                        |
|         | 103.0             | 22,125                     | 37,700                        |
| No. II  | { 91.4            | 27,500                     | 42,750                        |
|         | 92.3              | 24,500                     | 30,000                        |
| No. III | 98.9              |                            |                               |

70 Example I was subjected to solution annealing after pressing, and gave the following results.

TABLE III.—PROPERTY RESPONSE OF EXAMPLE I TO SOLUTION ANNEALING

| Temperature,<br>° F. | Time | U.T.S.,<br>K.s.i. | Y.S.,<br>K.s.i. | Percent El. |
|----------------------|------|-------------------|-----------------|-------------|
| 2,175                | 1    | 78.5              | 65.0            | 2.0         |
| 2,175                | 2    | 73.7              | 58.9            | 1.7         |
| 2,175                | 4    | 79.4              | 56.3            | 2.7         |
| 2,175                | 16   | 56.9              | 41.5            | 1.2         |
| 2,200                | 2    | 74.5              | 52.9            | 2.2         |
| 2,200                | 4    | 70.3              | 47.9            | 1.9         |

TABLE IV.—HARDNESS RESPONSE TO SOLUTION ANNEALING—AIR COOLING

| Example I  | Temper-<br>ature, ° F. | Time | Hardness RB |       |        |
|------------|------------------------|------|-------------|-------|--------|
|            |                        |      | Before      | After | Change |
| Sample No: |                        |      |             |       |        |
| 1          | 2,175                  | 1    | 101         | 100   | -1     |
| 2          | 2,175                  | 2    | 102         | 97    | -5     |
| 3          | 2,175                  | 4    | 101         | 95    | -6     |
| 4          | 2,175                  | 8    | 100         | 93    | -7     |
| 5          | 2,175                  | 16   | 102         | 89    | -13    |
| 6          | 2,175                  | 32   | 101         | 88    | -13    |
| 7          | 2,200                  | 1    | 101         | 97    | -4     |
| 8          | 2,200                  | 2    | 99          | 94    | -5     |
| 9          | 2,200                  | 4    | 101         | 94    | -7     |
| 10         | 2,200                  | 8    | 101         | 90    | -11    |
| 11         | 2,200                  | 21   | 104         | 92    | -12    |

The following tests were made to show the superior strength of metal-coated beryllium powder over a typical surface-oxidized beryllium powder:

#### EXAMPLE V

##### Composition A

Nominal 11 micron beryllium powder was chrome-coated and vacuum hot-pressed at 2000° F. and 2000 p.s.i. yielding a density of 1.876 gr./cc. The powder and hot-pressed chemistries were:

| Constituent | Powder,<br>percent   | Hot-Pressed,<br>percent |
|-------------|----------------------|-------------------------|
| BeO         | 0.5<br>(X-ray diff.) | 4.59                    |
| C           | .274                 | .231                    |
| Fe          | .130                 | .110                    |
| Al          | .029                 | .040                    |
| Ni          | .016                 | .017                    |
| Si          | .031                 | .055                    |
| Mg          | .111                 | .095                    |
| Cr          | .190                 | .210                    |
| Be          | ( <sup>1</sup> )     | ( <sup>1</sup> )        |

<sup>1</sup> Balance.

##### Composition B

Ball milled beryllium powder, surface oxidized to a minimum of 4.25% BeO and containing no alloy coating was vacuum hot-pressed at 2000° F. and 2000 p.s.i. yielding a density of 1.892 gr./cc. Weighted average powder particle size per Coulter counter was 8.2 microns. The powder chemistry was:

|     | Percent |
|-----|---------|
| BeO | 4.25    |
| C   | .43     |
| Fe  | .163    |
| Al  | .097    |
| Ni  | .018    |
| Si  | .085    |
| Mg  | .118    |
| Mn  | .012    |
| Cr  | .015    |
| Co  | .001    |
| Cu  | .006    |
| Ag  | .001    |
| Be  | Balance |

The above examples were tested and showed the following results:

TABLE V

|               | U.T.S.<br>p.s.i. | Y.S.<br>p.s.i. | Elongation,<br>percent | PEL<br>p.s.i. |
|---------------|------------------|----------------|------------------------|---------------|
| Composition A | 104,000          | 56,700         | Nil                    | 22,125        |
| Composition B | 61,900           | 56,700         | 0.75                   | 7,500         |

TABLE VI

| Material      | Original Grain Size,<br>microns | Grain Size after<br>2,200° F., 2 hours |
|---------------|---------------------------------|----------------------------------------|
| Composition A | 7                               | 7                                      |
| Composition B | 9                               | 13.3                                   |

Other data substantiating the inhibiting effect of the beryllide film is listed below for Composition A.

| Hours at 2,175° F. | Original Size<br>in Microns | Final Size<br>in Microns | Final<br>Hardness, R <sub>b</sub> |
|--------------------|-----------------------------|--------------------------|-----------------------------------|
| 2                  | 7.5                         | 8.6                      | 97                                |
| 4                  | 7.5                         | 8.4                      | 95                                |
| 8                  | 7.1                         | 9.0                      | 93                                |
| 16                 | 7.3                         | 9.2                      | 89                                |
| 32                 | 7.4                         | 12.4                     | 88                                |

It appears that after sixteen hours, full solutioning of the beryllide occurs, as evidenced by the very slight change in hardness between 16 and 32 hours, and the beryllide has diffused into the beryllium matrix. Once the beryllide has diffused into the matrix, grain growth occurs. For example, note increase from 7.4 to 12.4 after 32 hours at 2175° F.

In view of the foregoing, it is apparent that there is provided a new and improved process for producing heat-treatable beryllium metal of superior mechanical properties without sacrificing the weight advantage of beryllium.

As set forth above, the process involves the coating of beryllium powders with a metal which will form a beryllide on the surface of each individual particle and at the interface of said particles when pressed under heat. This beryllide interface prevents grain growth of the beryllium metal, and reinforces the beryllium matrix by providing a beryllide network throughout the beryllium pressing, thus increasing the strength of the beryllium product.

This process provides a beryllium product with high strength, a high precision elastic limit, and a superior modulus of elasticity. The precision elastic limit relates to the dimensional stability of the metal and is equivalent to the amount of stress which will cause one millionth of inch permanent deformation.

As stated above, it is within the scope of this invention to utilize any metal for coating the powders which will form a beryllide on the surface of the powders when pressed.

As this invention may be embodied in several forms without departing from the spirit or essential characteristics thereof, the present embodiment is therefore illustrative and not restrictive, and since the scope of the invention is defined by the appended claims, all changes that fall within the metes and bounds of the claims or that form their functional as well as conjointly cooperative equivalents are therefore intended to be embraced by those claims.

I claim:

1. A beryllium metal shape consisting essentially of bonded beryllium particles of a size of from 4 to 74 microns, each of said particles being coated with a beryllide of a metal selected from the group consisting of chromium, copper, nickel, columbium, molybdenum, cobalt and iron.

2. A beryllium metal shape as set forth in claim 1 wherein the particles are of a size of from 4 to 15 microns.

3. A beryllium metal shape as set forth in claim 1 wherein the beryllide coating has a thickness of up to 50 angstroms.

#### References Cited

##### UNITED STATES PATENTS

|           |         |            |          |
|-----------|---------|------------|----------|
| 3,294,530 | 12/1966 | Storchheim | 75—212 X |
| 3,150,975 | 9/1964  | Beaver     | 75—214   |

##### FOREIGN PATENTS

|         |         |                |
|---------|---------|----------------|
| 522,463 | 6/1940  | Great Britain. |
| 527,618 | 10/1940 | Great Britain. |

CARL D. QUARFORTH, Primary Examiner.

A. J. STEINER, Assistant Examiner.